

Patented June 1, 1926.

1,587,271

# UNITED STATES PATENT OFFICE.

MURRAY C. BEEBE AND ALEXANDER MURRAY, OF CINCINNATI, OHIO, ASSIGNEES TO  
THE WADSWORTH WATCH CASE COMPANY, OF DAYTON, KENTUCKY, A CORPORA-  
TION OF KENTUCKY.

## NATURAL-RESIN PHOTOGRAPHIC MEDIUM AND PROCESS.

No Drawing.

Application filed November 27, 1922. Serial No. 603,713.

The present invention relates to a photographic medium and process employing a natural resin, preferably a selected asphaltum, as the main base for the photographic medium. The invention or discovery comprises the features and steps hereinafter more fully described and claimed.

The primary purpose of the invention is to provide a sensitized medium in which the main base is a natural resin, preferably asphaltum, bitumen, or the like. A further object is to provide a sensitized asphaltum medium for photographic purposes which will print rapidly in a photographic operation, which will work with marked uniformity, which can be readily compounded and applied, and which provides a thoroughly practicable medium and process, available for all kinds of photographic purposes, etching, lithography, etc.

Examples are hereinafter given which will enable the invention to be understood and practiced.

Of the natural resins, it is preferred to employ the more sensitive parts of commercial asphaltum.

It is not necessary to describe the preliminary steps for separating the more sensitive parts of commercial asphaltum by means of ether, etc., as this procedure is well known, being fully described in existing literature. We have increased the sensitivity of asphaltum to a practical everyday uniformity; have removed the chemical complexity that has heretofore been associated with asphaltum developments and have made our process applicable to the various demands of all the industries which require a multiplication of illustrations.

Our process makes possible the production of printing surfaces from continuous tone negatives without recourse to an aquatint grain, reticulation, screens, etc. It also includes advanced developing steps, all of which insure great uniformity in practical results without being limited to absolutely exact exposures. It brings about an accurate reproduction of the tonal gradation and detail of the original and an ease and simplicity of manipulation which have not been reached heretofore. It is especially available for all lithographic purposes and is found to cooperate very well with screenless litho-processes. There is an advanta-

geous control factor in developing and the process is also available for the production of relief and intaglio printing plates, being of service in all the arts for contact exposures or optical projection. Under the usual arc-lamp source of illumination found in process engraving establishments the exposures may range from one-half minute to five minutes at the outside.

The sensitizer for asphaltum which we use is made up as follows:

|                               | Per cent. |
|-------------------------------|-----------|
| Ethyl methyl ketone           | 22        |
| Iodoform                      | 12        |
| Solvent naphtha               | 65½       |
| Concentrated ammonium hydride | 70<br>½   |

and the photographic medium or coating which we use consists of:

|                 | Per cent. |
|-----------------|-----------|
| Asphaltum       | 10        |
| Solvent naphtha | 40        |
| Benzine         | 25        |
| Sensitizer      | 25        |

Such a coating is flowed or otherwise applied to a grained or any desired smooth surface, allowed to drain and dry. The coated surface is then exposed to a luminous image by contact or by optical projection for from one-half minute to four minutes according to the character of the image. After the exposure the print is developed with

|                   | Per cent. |
|-------------------|-----------|
| Oleic acid        | 50        |
| White mineral oil | 50        |

by applying the same in a gentle manner and rubbing softly with any suitable medium. When completely developed the print is rinsed with dilute ammonia and then with water.

As heretofore stated, we do not limit ourselves to these specific formulas, materials, or procedure exemplified for the process is susceptible of wide variation, without sacrificing its great rapidity, to meet the exigencies of almost unlimited demands for speedy and simple reproduction of illustrations in the field of the graphic arts.

In specially referring to asphaltum, we do not exclude, but definitely include all classes of substances, known as natural res-

ins, etc., with which our sensitizer will co-operate to produce a highly sensitive actinic medium. Additional examples of natural resin which may be employed are gum kauri, 5 rubber, manila, congo, gutta percha, rosin, zanzibar, copal, etc. These materials may be used in the same manner as asphaltum, and in the proportions stated with respect to asphaltum. While the use of asphaltum 10 is preferred, gum kauri and rubber give good results. The other examples listed give fair results, but, as stated, asphaltum is preferred.

We have also found that the use of iodine, 15 heretofore proposed produces an unstable sensitizer. To be practical the iodine compounds, such as iodoform and a diluting neutral solvent, must not seriously affect the asphaltum while stored in the dark, they 20 must be freely soluble in the asphaltum, per contra, they must rapidly cause the asphaltum to become insoluble under the action of light, and finally, the unacted upon parts must be readily removed by a developing 25 solvent. Our sensitizer is stabilized by adding a small amount of ammonia. Halogen compounds or halides other than iodoform which do not react in the dark but are halogen liberating under the action of light so 30 as to produce insoluble compounds, are obviously included in our process.

Hydriodic acid and iodoform combined with asphaltum produce a highly sensitive 35 coating. To this may be added a small amount of ammonia which tends to stabilize the coating, or varnish. Before using the varnish, the ammonia preferably is neutralized. The composition may comprise: Hydriodic acid, 10%; iodoform, 20%; asphaltum, 40 79%; ammonia, a small amount.

Colloidal sensitizers, such as the following, 45 in some instances, produce great sensitivity and result in markedly shortening exposures to as short a time as ten seconds. These are exemplified by the following: 4.2 gms. lead triethyl iodide in 30 cc. benzene; 3.0 gms. asphaltum in 15 cc. solvent naphtha, and 3.0 gms. iodoform in 20 cc. ethyl methyl ketone. Such a sensitizer is also very stable 50 making possible its storage for a day without practical deterioration in contrast to unstable sensitizers, which often, spoil in a few hours. Reversals may be produced by using developing solvents that only act on the parts which have been exposed to the 55 light in any desired manner.

Our process, as already stated is applicable 60 to a multitude of uses, among them we may further specifically mention the production of screenless grained litho-plates; for line engraving on zinc, copper, etc., for relief printing; for half-tone purposes, such as monochrome or color separation plates; intaglio uses like photo and roto-gravure, in 65 one or more colors, etc, etc.

The procedure, in printing on our coating by means of electric light follows well known steps which need not be specifically described. The process has been referred to as being applicable to contact and projection printing, by inference, being restricted to same size subjects. We do not confine ourselves to such limitations but include all kinds of enlargements needed in lithographic or other poster work, from half-tone or continuous tone negatives, etc. The treated and selected asphaltum which we use is of itself very slightly sensitive to light, but as stated it is not sufficiently sensitive alone to serve any practical purposes. 70 75 80

In addition to our finding that iodine produces an unstable sensitizer we have also found that the use of iodine heretofore proposed as a sensitizer, cannot be accurately so classed because its action is to merely render the asphaltum less soluble. To become practical as a sensitizer iodine must be used in a combined form, from which, through the action of light, iodine will be liberated from the iodine compounds such as iodoform etc. 90 95

What we claim is:—

1. An asphaltum photographic process, consisting in combining a selected asphaltum with a colloidal halide, subjecting the same to a luminous image, and in subsequently 95 developing the print by means of a suitable solvent to remove variable soluble parts of the impressed image.

2. A resinous photographic process which comprises combining a slightly sensitive 100 natural resin as the main base of a photographic medium with a small percentage of a halogen-liberating sensitizer, subjecting the sensitized medium to a source of illumination, and subsequently developing the same 105 by means of a suitable solvent.

3. A photographic process, consisting in combining an asphaltum with a solvent, in adding thereto a halogen liberating agent and a suitable solvent, in coating a surface 110 therewith, in subjecting the coated surface to a luminous image, in developing the image and in finally rinsing the same.

4. A rapid photographic process, consisting in using a slightly sensitive asphaltum 115 with a solvent, in adding a sensitizer and solvent which is non-reacting on the asphaltum in the dark but which forms an actinic medium highly sensitive to light, in subjecting a coating of such medium to a luminous 120 image, and in subsequently developing the same.

5. A photographic process consisting in combining solvents with a natural resin taken as the main base of a photographic 125 medium, sensitizing the solution by combining therewith an iodine compound and a solvent yielding a stable mixture which will not deteriorate in the dark, printing by means of a variably luminous image on 130

a surface coated with said mixture, and developing the print.

6. The process of producing an actinic sensitizer for natural resins, which comprises combining iodoform, ethyl methyl ketone, a suitable solvent, and a trace of concentrated ammonium hydroxide.

7. The process of producing an actinically sensitive coating which comprises combining with asphaltum a colloidal halide in the presence of co-operating solvents.

8. A photographic process comprising forming a light-sensitive medium of a natural resin employed as the main base of a photographic medium by sensitizing the same with a halogen-liberating agent to form a stable mixture, applying a coating of said mixture to a grained metallic plate, exposing the coating to a luminous image, and developing with a suitable solvent.

9. A process of producing a stable, light-sensitive medium which comprises incorporating in a natural resin such as asphaltums, bitumens, asphaltites, etc., taken as the main base of the medium, and a solvent, a halogen-liberating compound which remains stable in such medium during storage.

10. The process of producing an actinically sensitive medium which comprises mixing together 10% asphaltum, 40% solvent naphtha, and 25% benzine; and incorporating therewith a solution comprising a halogen compound, such solution constituting approximately 25% of the sensitized medium.

11. A photographic medium consisting of approximately the following: 75% asphaltum solution; 25% sensitizing medium consisting of approximately 34% iodoform and ethyl methyl ketone and 66% solvent.

12. A photographic medium, comprising

a natural resinous compound as a main base, and a halogen-liberating sensitizer incorporated therein.

13. A photographic medium, comprising a slightly sensitive natural resinous compound as a main base, and a sensitizer incorporated therein comprising a light-sensitive metallic halide.

14. A photographic medium, comprising a slightly sensitive natural resinous compound as a main base, and a sensitizer incorporated therein comprising a light-sensitive colloidal metallic halide and a halogen-liberating organic compound.

15. A photographic medium, comprising a slightly sensitive natural resinous compound as a main base, and a sensitizer incorporated therein comprising a light-sensitive metallic halide and iodoform.

16. A photographic medium, comprising a selected light-sensitive asphaltum, and a sensitizer incorporated therein comprising a halogen-liberating compound.

17. A photographic medium, comprising a selected light-sensitive asphaltum, and a sensitizer incorporated therein comprising a light-sensitive metallic halide and a halogen-liberating organic compound.

18. A photographic medium, comprising a selected light-sensitive asphaltum, and a sensitizer incorporated therein comprising a light-sensitive metallic halide and iodoform.

19. A photographic medium, comprising a selected light-sensitive asphaltum and a sensitizer incorporated therein comprising iodoform.

In testimony whereof we affix our signatures.

MURRAY C. BEEBE.  
ALEXANDER MURRAY.